

1,017,969.

R. T. HARRIS.  
METHOD OF CASTING METAL.  
APPLICATION FILED JAN. 11, 1910.

Patented Feb. 20, 1912.

3 SHEETS—SHEET 1.

Fig. 1.



Fig. 2.



Witnesses.

*L. M. Daugler*  
*George A. Neubauer.*

Russ T. Harris, Inventor.

*By* *A. J. Daugler* *Attorney.*

R. T. HARRIS.

## METHOD OF CASTING METAL.

APPLICATION FILED JAN. 11, 1910.

1,017,969.

Patented Feb. 20, 1912.

3 SHEETS—SHEET 2.



### Witnesses.

J. M. Daugler.  
George A. Neubauer.

Inventor.

Russ J. Harris

Attorney,

1,017,969.

R. T. HARRIS.  
METHOD OF CASTING METAL.  
APPLICATION FILED JAN. 11, 1910.

Patented Feb. 20, 1912.

3 SHEETS—SHEET 3.



R. T. Harris Inventor.

Witnesses.  
J. M. Daugler  
George C. Neubauer.

By *G. J. Daugler* attorney.

# UNITED STATES PATENT OFFICE.

REESE T. HARRIS, OF BUFFALO, NEW YORK.

## METHOD OF CASTING METAL.

1,017,969.

Specification of Letters Patent. Patented Feb. 20, 1912.

Application filed January 11, 1910. Serial No. 537,522.

To all whom it may concern:

Be it known that I, REESE T. HARRIS, a citizen of the United States, residing at Buffalo, in the county of Erie and State of New York, have invented a certain new and useful Improved Method of Casting Metal, of which the following is a specification.

This invention relates to improvements in the art of casting metals and particularly to 10 the method of casting steel charging boxes and the like.

The principal objects of the invention are to materially cheapen the cost of casting by simplifying the operation and increasing the 15 rapidity, and to produce a casting of even and uniform firmness of metal which is not distorted from its regular shape or cracked in cooling and is provided with comparatively smooth surfaces.

20 For a full understanding of the nature and character of this improved method of casting metals, reference is to be had to the accompanying drawings in which a preferred adaptation of a mold capable of carrying out the method is shown.

Figure 1 is a transverse section through the mold. Fig. 2 is a transverse section through the mold similar to Fig. 1, but including the metal casting and illustrating 25 the metal core partially withdrawn from the mold. Fig. 3 is a top plan view of the improved mold. Fig. 4 is a central longitudinal section through the mold on line *a* *a*, Fig. 3. Fig. 5 is a fragmentary horizontal 30 longitudinal section through the mold on line *b* *b*, Fig. 4. Fig. 6 is a transverse section through the wooden pattern.

The improved mold utilized in this method constitutes the subject matter of a 40 companion application filed October 11, 1911, Serial No. 654,162.

In referring to the drawings in detail like numerals designate like parts.

The mold, briefly, consists of a drag, a 45 pattern and a collapsible metal element which forms both the cope and core. The drag has a flask 1 and a wooden pattern 2 which forms the exterior contour of the metal casting and is fitted in the flask 1 in 50 the usual manner. Green sand is then tamped into the flask around the pattern to secure the imprint of the pattern and form the lower green sand portion 3 of the mold.

The interior contour of the box is formed 55 by a metal element which is fitted on the flask 1 after the mold portion 3 is completed

and the wooden pattern 2 is withdrawn. This metal element is preferably constructed of two parts or members which are hinged together so that they can collapse 60 or fold together. The members are practically similar in size and shape but extend oppositely and are opposed to each other so that when in open position the metal element will be of a dished or barrel like form. 65

The members each consist of a lower approximately horizontal inwardly extending portion 4, a vertical medial portion 5 and a horizontal outwardly extending top flange portion 6. 70

The hinges for connecting the members consist of lugs 7 which extend up from the top surfaces of the horizontal portions 4 near the inner margins thereof and lap each other, and hinge pintles 8 which are loosely 75 fitted through eye openings in the lugs.

Two hinges each consisting of three lugs and a pintle are preferably utilized, each of which is located near one end of the metal element. 80

It will be noted that the junction of the lower horizontal portion 4 and the medial vertical portion 5 is of a rounded form. The object of this is to give a similar rounding contour to the interior of the casting 85 and also to enable the members of the metal element to be easily turned on their hinges and withdrawn from the casting.

When the metal element is in position to form the interior contour of the casting as 90 shown in Fig. 1, the lower inner edges of its members butt closely together, so that an extremely smooth and practically unbroken surface is presented to the molten metal as it flows in. 95

The metal element is collapsed and withdrawn after the molten metal is poured in the mold by means of a crane or other suitable machine (not shown) from which lifting hooks 9 depend. 100

A fragment of one of the hooks 9 is shown in dotted lines in Fig. 2.

The two members of the metal element or core are held in their separated position as shown in Fig. 1, by bridge bars 10 which extend transversely between members and are connected at their respective ends to the members by pins 11 which pass through holes 12 in the bridge bars and holes 13 in raised cross ribs 14 on the top flanged portions of 110 the members. Each bridge bar has a central upwardly extending lug 15 which is pro-

vided with an opening 16 in which one of the hooks 9 engage. Each of the bridge bars is additionally connected to one of the members of the metal element or core by a link 17 which is pivoted at its inner end by a pin 18 to the bridge bar at a point vertically below the opening 16 in the lug 15, see Fig. 1. The outer end of the link is pivoted by a pin 19 to an inwardly projecting lug 20 located near the top of the vertical medial portion 5 of one of the members.

The members of the metal element or core are each stiffened and strengthened on their inner surface by longitudinal and transverse ribs 21 and 22.

15 The ends of the core are closed by end pieces which are formed of sand inserted in place between the end margins of the members of the metal element or core when in 20 their separated position, as in Fig. 1.

25 As the charging box designed to be cast with this improved process and the mold shown in the accompanying drawings has a slotted end and a plain end, one of the end pieces is formed in two separated sections 23 and 24 which are fitted together as shown in Fig. 5, and shaped to leave the necessary slot in the slotted end and the other in one solid piece 25.

30 The pouring hole 26 is located at one end of the sand portion 3 of the mold and the vent hole 27 at the opposite end of said sand portion.

This improved process is mainly used in 35 casting thin, narrow elongated pieces of dished form which are difficult to cast in the ordinary manner with sand cores and practically impossible to cast with solid metal cores.

40 In carrying out this process the wooden pattern 2 is first placed on the flask 1 and green molding sand is then rammed into the space between the flask and pattern to form the lower sand portion 3 of the mold.

45 The pattern is withdrawn after the sand portion 3 is completed and the metal element or core is fitted on the flask and the sand end pieces placed in the ends of the metal element or core. The molten metal which forms 50 the casting is now poured in the pouring hole 26 until it runs out of the vent 27 at the opposite end. After the casting is poured, the metal element is collapsed and lifted very quickly from the casting and before the 55 casting has cooled beyond the surface hardening of the metal.

By removing the metal element the interior surface of the casting is completely exposed to the air so that it may cool evenly 60 and shrink or contract freely. This prevents any distortion or cracking of the metal and produces a casting of regular form and uniform firmness of metal.

To prevent sudden chilling of the molten 65 metal, the metal element is heated in any

well known manner before the metal is poured in the flask, for instance, a fire may be built in the metal element.

The metal element or core is preferably constructed of cast iron and it is washed 70 with a composition of graphite and fire clay or any other suitable composition for producing a smooth non-adhesive surface to contact with the molten metal. The collapsing of the metal element also breaks up the 75 sand end pieces of the core, so that the casting when sufficiently cooled can be easily removed from the lower sand portion 3 of the mold. But one flask is required with this construction as the metal element serves 80 not only as a core and a cope but also as the entire top portion of the mold.

The wooden pattern 2 is provided on its bottom with two parallel longitudinal ribs 28 which press channels 29 in the surface of 85 the lower sand portion 3 of the mold. These channels constitute gates for the flowing molten metal and also serve to form corresponding parallel longitudinal ribs 30 on the bottom of the casting. After the wooden 90 pattern is removed converging grooves or channels 31 are formed which extend from the ends of the channels 29 to the pouring hole or gate.

The flask and metal core are pinned to 95 each other so that they will register properly together. This is accomplished by providing flanges 32 or the like on the outer margins of the top portions of the flask sides and providing such flanges with vertical 100 pins which are adapted to enter openings in the lateral extensions 34 of the metal core.

End plates 35 are fitted on the ends of the flask over the ends of the mold and are held 105 in place by weights or clamps. These plates serve to close the top ends of the flask as the core is not as long as the flask and also prevent the sand from being forced out over the top by the molten metal as it is poured in.

One of the principal purposes for which 110 this improved method is utilized is in the casting of charging boxes from open hearth and Bessemer and other forms of steel and directly from the ladle, the iron being converted into steel and then carried to and 115 poured into the mold while still in a molten state.

In carrying out this improved process of casting metal, the lower or sand portion of the mold is first formed, the metal element, 120 the outer surface of which has been coated with the non-adhesive composition as before described, is fitted in place on the flask, the sand end pieces are fitted in place, the metal element is heated to about the desired temperature, the molten metal is poured in to 125 form the casting, and the metal element is immediately collapsed and lifted from contact with the casting.

The principal features of this improved

method of casting metal residue in simplifying the operation of producing the necessary mold by dispensing with a sand core and a cope and utilizing in lieu thereof a metal element which forms a permanent core and cope, in heating the metal element to prevent sudden chilling, in arranging this metal element so that it can be immediately withdrawn as soon as the metal is poured, which exposes the hot casting to the even and uniform and comparatively quick cooling action of the surrounding air, and permits it to shrink and contract freely while cooling to prevent distortion or cracking, in greatly increasing the capacity of production of the molds and castings and in producing perfect undistorted, uncracked and regular castings of even firmness of metal, with smooth surfaces and without blow holes or defects.

I claim.

1. A method of casting metals which consists in pouring the molten metal in a mold composed in part of non-friable metal and in part of friable material and then when the metal of the casting solidifies collapsing the non-friable metal part of the mold and breaking up the friable part.

2. The hereinbefore described method of casting metals consisting in first preparing a mold including a metal element and separate sand elements, heating the metal element to prevent sudden chilling of the molten metal, pouring the molten metal in the

mold, and then quickly removing the metal element of the mold, and simultaneously breaking up some of the sand elements to completely expose the interior of the hot casting to the atmosphere.

3. A method of casting metals which consists in pouring the molten metal in a mold composed in part of non-friable metal and in part of friable material and then when the metal of the casting solidifies simultaneously collapsing the non-friable part of the mold and breaking up the friable part.

4. A method of casting metals which consists in pouring the molten metal in a mold composed in part of non-friable metal and in part of friable material and then when the metal of the casting solidifies collapsing the non-friable part of the mold and by said collapsing crushing and breaking up the friable part.

5. A method of casting metals which consists in pouring the molten metal in a mold having a composite collapsible core of non-friable metal and friable material so constructed that the collapsing of the core portion of non-friable metal will crush and break up the portion of friable material and then when the metal of the casting solidifies collapsing and removing said core.

REESE T. HARRIS.

Witnesses:

W. H. EBSORY,  
L. M. SANGSTER.